

# United States Patent Office

3,340,047  
Patented Sept. 5, 1967

## 1

3,340,047

### FORGEABLE CORROSION-RESISTING STEEL WITH HIGH NEUTRON-ABSORPTION CAPACITY

Karl Gerhard Sune Persson, Kedjeasen, Paul Helmer Lindroth, Soderfors, and Lars Ivar Hellner, Karlskoga, Sweden, assignors to Aktiebolaget Bofors, Bofors, Sweden, a corporation of Sweden  
No Drawing. Filed Nov. 26, 1963, Ser. No. 326,216  
Claims priority, application Sweden, Dec. 8, 1962,  
13,250/62

6 Claims. (Cl. 75—126)

The present invention relates to a forgeable, corrosion-resistant steel with a high neutron-absorption capacity. Such a steel is well suited for the manufacture of control rods for nuclear reactors and radiation-protection screens.

In a nuclear reactor, the development of energy is directly affected by the flow of neutrons, and it is therefore necessary to be able to control this flow. Such control is usually carried out by inserting control rods into the flow, which have a screening effect, owing to their containing a substance which has a high absorption cross-section for neutrons, and such a substance is boron which, contrary to most other substances with the corresponding properties, is also cheap. The active constituent in boron is the isotope B<sup>10</sup>, of which there is a content of 18.9% in natural boron.

With consideration to the strength required, however, it is not possible to manufacture control rods of pure boron or any simple chemical compound thereof, and it is usually necessary to use boron as an alloying element in steel, in order to obtain the strength required. However, the quantity of boron which can be added is limited, owing to the fact that large boron contents have a very detrimental influence on the hot-working properties, and when unalloyed steel is used, a boron content of not more than approx. 2.5% can be permitted, if satisfactory forgeability is to be obtained. It is known, however, that by adding aluminum or silicon at the same time, the boron content in a steel alloy can be increased to a maximum of 4.5%, while fairly acceptable hot-working properties are still maintained.

However, steels of the above-mentioned types have comparatively poor corrosion resistance, and for this reason often cannot be used. Attempts have therefore been made to use boron as an alloy in a basic material consisting of austenitic, stainless steels of the type 18% chrome-8% nickel. In these steels, however, the hot-working properties have been lost entirely if the boron contents have exceeded 2%.

It has now proved that with a steel according to the present invention, good hot-working properties can be maintained even with boron contents of up to approx. 5%, at the same time as a corrosion resistance is obtained which is considerably better than that of unalloyed steel.

The new forgeable, corrosion-resistant steel with a high neutron-absorption capacity, is characterized according to the present invention in that it contains

|                 |       |
|-----------------|-------|
| Percent         |       |
| Carbon, maximum | 0.15  |
| Chrome          | 15-30 |
| Boron, maximum  | 5     |

and titanium in such a quantity that, when accounted for as weight percent, it amounts to at least

$$3.1 \times (\text{weight percent boron}) - 5.8$$

in addition to which the type of steel in question has normal contents of silicon and manganese, and impurities such as phosphorous and sulphur.

## 2

In the following table, some examples are given of steels according to the present invention.

| 5  | Steel No. | Contents, percent |        |          |       |
|----|-----------|-------------------|--------|----------|-------|
|    |           | Carbon            | Chrome | Titanium | Boron |
| 10 | 1.....    | 0.03              | 25.1   | 4.5      | 2.4   |
|    | 2.....    | 0.04              | 25.1   | 6.0      | 3.0   |
|    | 3.....    | 0.04              | 25.1   | 5.4      | 3.5   |
|    | 4.....    | 0.03              | 25.3   | 6.6      | 3.7   |
|    | 5.....    | 0.03              | 25.4   | 6.8      | 3.7   |
|    | 6.....    | 0.03              | 25.4   | 7.3      | 3.8   |
|    | 7.....    | 0.03              | 25.4   | 7.4      | 4.0   |
|    | 8.....    | 0.04              | 24.0   | 8.0      | 4.4   |

15 In addition to the constituents mentioned above, the steels also have somewhat varying contents of silicon and manganese, although not more than 2% of each, as well as normal impurities such as phosphorous and sulphur.

20 All of the above-mentioned steels proved to have good hot-working properties, and could be forged from ingots into bars without any major difficulties. The forging was then carried out within the temperature range of 950°-1100° C.

25 All of the steels listed in the table also showed extremely good corrosion resistance. In order to obtain the good corrosion resistance desired it proved necessary to allow the chrome content to amount to more than 15%.

29 Keeping the carbon content low, below 0.15%, facilitates the hot-working, and because of the comparatively high chrome content, the steel will be ferritic within the whole of the temperature interval which will come into question.

33 The major portion of the boron used should be in the form of titanium boride, but it is not possible, however, to foresee theoretically the minimum quantity of titanium which is required in order to obtain satisfactory hot-working properties. The relation between the minimum titanium content and the boron content has therefore been found as the result of a great number of experiments.

37 What is claimed is:

38 1. Forgeable, corrosion-resistant steel, having a high neutron-absorption capacity, consisting essentially of:

|                                                                     |       |
|---------------------------------------------------------------------|-------|
| Percent                                                             |       |
| 45 Carbon, maximum                                                  | 0.15  |
| Chromium                                                            | 15-30 |
| Boron, maximum                                                      | 5     |
| Titanium in weight percent of at least 3.1 × (weight percent boron) | — 5.8 |

50 balance essentially iron.

51 2. Steel in accordance with claim 1 which contains

|                     |   |
|---------------------|---|
| Percent             |   |
| 55 Silicon, maximum | 2 |
| Manganese, maximum  | 2 |

56 3. Steel in accordance with claim 1, wherein the carbon content is a maximum of 0.10%.

57 4. Steel in accordance with claim 2, wherein the carbon content is a maximum of 0.10%.

58 5. Steel in accordance with claim 1, wherein the chromium content is 18-28%.

59 6. Steel in accordance with claim 2, wherein the chromium content is 18-28%.

## References Cited

### UNITED STATES PATENTS

1,493,191 5/1924 Golyer ----- 75—126

70 70 DAVID L. RECK, Primary Examiner.  
P. WEINSTEIN, Assistant Examiner.